

Patented Jan. 12, 1926.

## UNITED STATES PATENT OFFICE.

ADOLF FÖRSTER, OF KULLEBUND, NEAR CHRISTIANIA, NORWAY.

## MANUFACTURE OF ARTIFICIAL WOOD.

No Drawing.

Application filed October 17, 1923. Serial No. 669,186.

*To all whom it may concern:*

Be it known that I, ADOLF FÖRSTER, of Kullebund, near Christiania, Norway, have invented certain new and useful Improvements in the Manufacture of Artificial Wood; and I do hereby declare the following to be a full, clear, and exact description of the invention, such as will enable others skilled in the art to which it appertains to make and use the same.

This invention has for its object a method for the manufacture of artificial wood in which a composition comprising saw dust, fillers and an animal glue (gelatine) is subjected to pressure.

An important feature of the present process as compared with hitherto known processes of this type consists therein that the glue is incorporated into the other constituents of the composition by means of moistening with a quite dilute solution of glue, which before application has been intimately mixed with a solution of a tanning or coagulating agent.

In the manufacture of artificial wood in accordance with the present invention one may for example proceed as follows:

90 parts by weight of saw dust and 10 parts by weight of chalk are thoroughly mixed so that the individual particles of saw dust are entirely enclosed in chalk.

This mixture of saw dust and chalk is moistened with a solution produced in the following manner:

7 parts by weight of ordinary glue (joiners glue) are dissolved in 90-95 parts by weight of water and when dissolution has been effected 5-10 parts by weight of acetic acid (according to the quality of the glue) is added. This solution is thoroughly mixed with an aqueous solution of potassium bichromate in a quantity of from 2-3 per cent of the weight of the dry glue.

To the first mentioned mixture of saw dust and chalk is now added so much of the chromate-glue solution (suitably about 35-45 kilogrammes) that the mass becomes well moistened throughout but not more. The moistened mass is worked thoroughly through preferably in full daylight and is thereupon brought into moulds (preferably with smooth surfaces), which are suitably constructed of iron and is subjected for some time (for example a couple of hours) to a very high pressure. The shaped objects are thereupon removed from the moulds and

dried in the air. In the described example the dry product for each kilogram of saw-dust-chalk mixture will not contain more than about 0.03 kilogrammes of glue. 60

The completely dried product can be worked as natural wood with saw, plane, drill and other wood-working tools. The material can also be glued (joined), coloured, painted and fastened by nails or 65 screws.

Instead of chalk other mineral fillers of a low degree of hardness such as soap-stone, talcum may also be employed. The addition of acetic acid to the composition is not absolutely necessary but will in most instances produce the best results. The potassium bichromate can wholly or in part be substituted for by other substances, which have a tanning or coagulating effect upon gelatine, but 70 it has been found, that the best results are obtained by the use of a chromate or chromic acid as a hardener.

It is of great importance, that a dilute solution of glue is used so that the percentage of glue, which is incorporated into the composition by the moistening operation, is quite small.

Products produced according to this invention can be exposed to atmospheric influences without warping and without shrinking or cracking. It is only a little heavier than natural wood and floats on water. The product is insoluble in water and burns only when subjected to very high temperatures—high glow heat—and does not rot owing to the contained chemicals. The moist composition can be pressed directly upon veneer by placing the veneer in the bottom of the mould. The veneer cannot afterwards be loosened from the dry mass. Veneered plates produced in this manner are not subjected to the drawbacks frequently connected with natural wood which consist in warping and cracking of the wood 90 base. 95

The manufacturing costs of the artificial wood product is low. It is hard and has a great resistance against wear, and it can therefore with great advantage be used in steps of staircases, and in slabs of suitable size for wainscot, for floors etc. Reinforced with iron the material may be used to produce window frames and other objects. 105

Further this artificial wood can be used 110 in the manufacture of furniture and many other objects.

## Claims.

1. Method of manufacturing artificial wood comprising the steps of moistening a mixture containing saw dust and a soft mineral filler with a dilute solution of chrome-glue in which the percentage of glue is considerably less than 10 per cent thoroughly working the moistened mixture, moulding the resulting mass under a high pressure, maintaining the pressure for a considerable time and subjecting the moulded articles to drying.
2. Method of producing artificial wood according to claim 1 in which the dry saw dust composition is moistened with a chrome-glue solution to which acetic acid has been added.
3. Method according to claim 1 in which the moistened mass is pressed upon a reinforcing material.
4. Method according to claim 1 in which the mass is pressed upon veneer.

In testimony that I claim the foregoing as my invention, I have signed my name.

ADOLF FÖRSTER.